

# UNITED STATES PATENT OFFICE.

GILBERT H. THIME, OF CHICAGO, ILLINOIS.

## PLATING COMPOUND.

No. 839,148.

Specification of Letters Patent.

Patented Dec. 11, 1906.

Application filed March 8, 1906. Serial No. 304,892.

*To all whom it may concern:*

Be it known that I, GILBERT H. THIME, a citizen of the United States, and a resident of Chicago, Cook county, Illinois, have invented 5 certain Improvements in Plating Compounds, of which the following is a specification.

This invention relates to certain improvements in that class of compounds which are especially designed and adapted for employment in plating metal articles, and has for its object to provide a compound of this general character of a comparatively simple and inexpensive nature which shall be adapted 15 for ready and convenient use for imparting a substantial bright plate to metallic articles without the necessity of employing a plating-bath, whereby the compound is particularly well adapted for household and similar use 20 for plating faucets and similar articles of brass and iron.

The invention consists in a certain novel combination of the ingredients of the improved plating compound whereby the same 25 is capable of being prepared in a simple and inexpensive manner in powdered or comminuted solid form and is adapted for convenient application to the articles to be plated without requiring the employment of a bath, 30 as is ordinarily required for such work, all as will be hereinafter fully set forth.

The novel features of the invention will be carefully defined in the claims.

In preparing my improved plating compound I take of powdered or comminuted tin three and one-half parts, of powdered or comminuted lead four and one-half parts, and of mercury eight parts, by weight, and these ingredients I triturate in a mortar or 35 otherwise to form an amalgam of a dry and friable nature. In certain cases I have discovered that either by reason of impurities in the commercial mercury or by reason of lack of impurities therein or from other 40 causes a dry friable amalgam is not obtainable from these ingredients, and in such cases I add to the mass in the mortar a suitable proportion of antimony, which may vary from a mere trace to a proportion of 45 about one-half ounce to about eight pounds of the three first-mentioned ingredients, and the addition of the antimony in such suitable proportions imparts the desired dry friable 50 character to the resultant amalgam.

55 Of the friable amalgam thus produced I

then take sixteen parts, by weight, to which I add three and one-half parts, by weight, of sal-ammoniac, and these ingredients are also triturated to a dry powdered or comminuted condition and constitute the improved plating compound, which may be packed in suitable wood or other containers (not of metal) for use.

In the use of the improved plating compound for plating brass the article to be plated is first cleansed from grease and the like by being washed over with a solution composed of one part of salt, one part of vinegar, and two parts of water, after which the dry plating compound is rubbed over the cleansed surface of the article for plating the same. Usually for such plating it is necessary to apply about three coats of the plating compound to the surface, taking care to thoroughly cleanse the article after each coat, and to allow sufficient intervals between the plating operations for the compound to set upon the surface; but when the improved compound is properly applied it imparts a bright and durable plating to the brass and by reason of its inexpensive composition and ease and convenience of application is especially well adapted for household use for plating brass faucets and similar articles.

The improved compound is also well adapted for use in plating iron, and when employed for this purpose the mode of application above described is followed, except that in lieu of the salt and vinegar cleansing solution the metal to be plated is first cleansed with muriatic acid before application of the improved plating compound.

From the above description it will be seen that the improved plating compound is of an extremely simple and inexpensive nature and is capable of easy and convenient use for imparting a bright and durable plate to articles of brass and iron, and it will also be obvious from the above description that the improved compound is capable of some modification without material departure from the principles and spirit of the invention, and for this reason I do not desire to be understood as limiting myself to the precise proportion of the ingredients herein set forth in carrying out my invention in practice.

Having thus described my invention, what I claim, and desire to secure by Letters Patent, is—

1. The improved plating compound herein

described consisting of a dry comminuted or friable substance containing tin, lead, mercury and sal-ammoniac.

2. The improved plating compound herein described consisting of a dry comminuted or friable substance composed of tin, lead, mercury, sal-ammoniac and antimony.

In testimony whereof I have hereunto

signed my name, at Chicago, Illinois, this 6th day of March, 1906, in the presence of two subscribing witnesses.

GILBERT H. THIME.

Witnesses:

J. D. CAPLINGER,  
E. T. SPECHT.